

J. ASTON.

METHOD OF MAKING WROUGHT IRON.

APPLICATION FILED APR. 24, 1920.

1,412,823.

Patented Apr. 18, 1922.



# UNITED STATES PATENT OFFICE.

JAMES ASTON, OF PITTSBURGH, PENNSYLVANIA, ASSIGNOR TO A. M. BYERS COMPANY, OF PITTSBURGH, PENNSYLVANIA, A CORPORATION OF PENNSYLVANIA.

## METHOD OF MAKING WROUGHT IRON.

1,412,823.

Specification of Letters Patent. Patented Apr. 18, 1922.

Application filed April 24, 1920. Serial No. 376,247.

To all whom it may concern:

Be it known that I, JAMES ASTON, residing at Pittsburgh, Allegheny County, Pennsylvania, have invented a new and useful Improvement in the Methods of Making Wrought Iron, of which the following is a full, clear, and exact description, reference being had to the accompanying drawing, forming part of this specification, in 10 which—

The figure is a diagrammatic view showing one form of apparatus for carrying out my invention.

In my application, Serial No. 387,995, filed 15 November 14, 1919, for method of making wrought iron, I have described a method, in the preferred form of which the product of a steel-making process is granulated or comminuted and then mixed with slag, preferably by dropping the granules into a slag 20 bath, where a coherent mass or ball is formed.

I have found a simpler, cheaper and easier way of granulating and making a coherent 25 mass or ball, which consists in pouring the molten product of the steel-making process directly into the bath of slag of the proper characteristics. I have found that when a stream of steel is poured into a bath of 30 molten slag, it will become granulated, the granules dropping through the bath and cohering to form a mass or ball conforming generally to the bottom portion of the slag container, such as a slag ladle. It is therefore unnecessary under this invention to 35 granulate or comminute the steel in the air before it reaches the slag bath, since the molten metal will be granulated by the molten stream entering the slag bath. The granules 40 take the form of a sort of sponge, which is thoroughly intermingled with the slag, giving a mass or ball of these particles which weld together and form a ball ready for compressing. This is formed below the 45 surface of the slag bath which protects the metal from the air, and by making a sufficiently large ball or mass, I can roll the same after compressing directly into slabs or billets without repiling. These slabs or 50 billets may then be rolled, reheated and rolled into skelp, or other semi-finished or finished product.

In the drawing, in which I show diagrammatically one form of apparatus for carrying out my invention, 2 represents a slag heating furnace in which a puddling slag may be prepared. These slags are essentially iron silicates containing ferric oxide, ferrous oxide, silica, phosphoric oxide and manganese oxide with some alumina. The ferric oxide should be kept low, as it has a high oxidizing power in contact with metallic iron, the reaction producing ferrous oxide from the iron. Consequently, I preferably employ carbon on or in the slag bath 55 which may be in the form of crushed coke, carbon electrodes, etc., to keep the percentage of ferric oxide low and to reduce the same to some extent. The coke or other carbon blanket over the slag will, of course, be held back when the slag is poured into the ladle 60 3 from this slag-heating furnace. The ladle 3 may be mounted on a truck 4, by which it may be carried under a pouring stand, indicated at 5. The product of the steel-making operation may be taken from a steel-making furnace, consisting of a Bessemer converter, an open-hearth furnace, an electric furnace, or any other desired apparatus 65 for making molten steel. 70

A suitable charge for a large ball, say 2,000 pounds, is tapped out of this furnace into a ladle 7, which ladle may then be taken by an overhead crane to the pouring stand directly above the ladle of slag. The height 75 is preferably about eight feet for the drop of the stream of metal. This, however, may be varied within wide limits in both directions, and the desired result obtained. The steel ladle is preferably a bottom-pour ladle. 80

The molten metal may be poured directly from the steel-making furnace without the use of a ladle, in which case, the necessary height of fall may be obtained by elevating the steel-making furnace or mounting it 85 above the pouring station. 90

When the stream of steel drops into the slag bath, it becomes granulated as it strikes and passes through the slag bath and forms a ball or coherent mass of welded particles, 100 thoroughly intermingled with the slag. This mass takes the general shape of the bottom of the slag ladle and lies under the surface of the slag, of which there is a sur-

plus over the amount necessary for intermingling with the metal in forming the ball.

After this operation, the surplus slag may be poured out by tipping the ladle, the slag 5 preferably passing through a screen 8, into a slag bucket or ladle 9, in the pit underneath the same. Instead of feeding the surplus slag into the slag receptacle by which it may be returned to the furnace, the surplus slag 10 may be poured directly back into the slag-melting furnace. The coherent ball of wrought iron is then taken out of the ladle to a squeezing apparatus 10, which is shown as of the "press" form, although it may be 15 of the rotary squeezer type or any other desired type. The "press" form is desirable, as the metal may thus be compressed into the desired shape, without turning or manipulating.

20 From the squeezing apparatus, the large ball is taken to a blooming mill and rolled at the same heat into slabs or billets. Or the bloom may be taken to a soaking pit for holding and equalizing its heat or for being 25 further heated prior to rolling it into slabs or billets. These slabs or billets may then be stored and passed through a continuous heating furnace to a skelp mill where they are rolled directly into skelp; or to another 30 mill to give any desired product, such as wire, sheets, etc.

It will be noted that with this large ball, thorough distribution and dissemination of the slag through the rolled mass is afforded 35 so that no cutting and repiling of muck bar, as in the usual puddling operation, is necessary.

The temperature of the slag is preferably sufficiently below that of the molten metal 40 entering it so that in the adjustment of the equilibrium of temperature between the slag and the metal, the granulated iron will solidify in the spongy mass or ball, on account of its being at the welding heat necessary for that purpose. The heat of the 45 slag may vary and the temperature of the ball may vary to a considerable extent, as it is taken out of the ladle or slag receptacle. The ball may be subjected to a soaking 50 pit operation to equalize the temperature through this mass after squeezing.

The excess slag from the ball which is poured through the grating into the excess slag receptacle may be returned to the slag-heating furnace. If this is done, however, I 55 have discovered that the slag should be revivified by the addition of silica. The forming of the ball introduces some iron oxide into the slag, thereby diluting the iron silicates so that to keep the slag of the proper physical and chemical characteristics, the 60 slag which is returned to the bath should be revivified by the addition of silica.

The formation of ferric oxide in the slag 65 may be retarded or prevented by keeping a

reducing atmosphere instead of an oxidizing atmosphere in the slag-melting furnace. The slag receptacle may consist of a large ingot mold and after the large ball or mass is formed and the excess slag removed, the mass may be compressed or squeezed in this mold and then taken to a soaking pit where the heat is equalized through the mass, the compressed mass being then taken to the blooming mill.

70 Such a process is described in my copending application Serial No. 376,388, filed April 24, 1920.

The steel which I employ is preferably a low carbon steel, though the percentages of 80 metalloids in the steel may be varied widely without departing from my broad invention.

Many changes may be made in the apparatus employed, as well as in the steps of 85 my process, without departing from my invention. Within the scope of my claims, parts of my complete process forming sub-processes, may be used, without departing from my invention.

I claim:

1. The method of producing wrought iron, 90 consisting in pouring the molten substantially slagless product of a steel-making process into a slag bath, thereby comminuting the metal in the bath, and forming the 95 mixture into a coherent mass, substantially as described.

2. The method of producing wrought iron, 100 consisting in pouring the molten substantially slagless product of a steel-making process into a bath of puddling slag having the proper physical and chemical characteristics, thereby comminuting the metal in the 105 bath, and forming a coherent mass of mixed slag and metal below the surface of the slag in the bath, substantially as described.

3. The method of producing wrought iron, 110 consisting in pouring the molten substantially slagless product of a steel-making process into a bath of puddling slag having the proper physical and chemical characteristics, thereby comminuting the metal in the 115 bath, and forming a coherent partially shaped mass of slag and metal underneath the surface of the slag and corresponding to the shape of the lower part of the slag receptacle, substantially as described.

4. In the method of producing wrought iron, the steps consisting in providing a bath of an iron silicate slag of proper physical and chemical characteristics, pouring the molten product of the steel-making process into said bath, thereby comminuting the metal in the bath, and forming a coherent mass of mixed metal and slag therein, substantially as described.

5. In the method of producing wrought iron, the steps consisting of feeding the molten products of a steel-making process into a bath of slag of the proper physical 130

and chemical characteristics for making wrought iron, comminuting the steel after it strikes the slag bath, and causing the metal granules to contact with each other 5 below the surface of the slag bath while at welding temperature, thereby forming a coherent mass or sponge beneath the surface of the slag bath, substantially as described.

6. The method of producing wrought iron, 10 consisting in pouring the molten substantially slagless product of a steel-making process into a slag bath, thereby comminuting the metal in the bath, forming the mixture into a coherent mass, freeing the mass 15 from the surplus slag, and compressing it, substantially as described.

7. In the method of producing wrought iron, the steps consisting of pouring a stream of the molten product of a steel-making 20 process into a bath of slag of the proper characteristics, forming a spongy shaped mass of mixed steel and iron in the bottom portion of the slag receptacle, removing the mass from the receptacle, and compressing 25 it, substantially as described.

8. In the method of producing wrought iron, the steps consisting of maintaining a molten bath of iron silicate slag of the proper characteristics for making wrought 30 iron, preventing or retarding the formation of ferric oxide therein, feeding successive portions of the slag into receptacles, feeding the molten product of a steel-making process into the slag in the receptacle, and forming 35 a spongy mass of slag and metal therein, substantially as described.

9. In the method of producing wrought iron, the steps consisting of maintaining a molten bath of iron silicate slag of the proper characteristics, preventing or retarding 40 the formation of ferric oxide in the bath, feeding out a portion of the bath into the slag receptacle, pouring the molten product of a steel-making process into the slag in the receptacle, thereby comminuting the same and forming a wrought iron sponge in 45 the bottom of the receptacle, and then removing and compressing the same, substantially as described.

50 10. In the method of producing wrought iron, the steps consisting of pouring the molten product of a steel-making process into a receptacle containing a bath of slag of the proper characteristics to make 55 wrought iron, forming a large wrought iron ball or mass therein, squeezing or pressing the same, and rolling it directly into slab or billet form, substantially as described.

11. In the method of producing wrought 60 iron, the steps consisting of pouring the molten product of a steel-making process into a receptacle containing a bath of slag of the proper characteristics to make wrought iron, forming a large wrought iron ball or mass therein, squeezing or pressing 65

the same, and then rolling the slab or billet into the desired product, substantially as described.

12. In the method of producing wrought iron, the steps consisting of pouring the 70 molten product of a steel-making process into a receptacle containing a bath of slag of the proper characteristics to make wrought iron, forming therein a large mass or puddle ball of such a size as not to require repiling, and rolling the same directly 75 into the desired product, substantially as described.

13. In the method of producing wrought iron, the steps consisting of pouring the 80 molten product of a steel-making process into a receptacle containing a bath of slag of the proper characteristics to make wrought iron, forming therein a large mass or puddle ball of such a size as not to require repiling, and squeezing and rolling 85 the same directly into the desired product, substantially as described.

14. In the process of making wrought iron by mixing the molten product of a 90 steel-making process with slag of the proper characteristics for making wrought iron, the step consisting of removing the surplus slag from the ball or mass, and revivifying the slag, substantially as described. 95

15. In the process of making wrought iron by mixing the molten product of a steel-making process with slag of the proper characteristics for making wrought iron, the step consisting of removing the surplus slag 100 from the ball or mass, and revivifying the slag by adding silica, substantially as described.

16. In the method of producing wrought iron, the steps consisting of maintaining a 105 molten bath of slag of the proper characteristics for making wrought iron, withdrawing a portion thereof into a slag receptacle, feeding thereto the molten product of a steel-making process to form a spongy mass 110 or ball of wrought iron, freeing the mass from the surplus slag, and revivifying and returning said slag to the general bath of molten slag, substantially as described.

17. As a new article of manufacture, a 115 shaped spongy mass of wrought iron formed of the granulated product of a steel-making process mixed with slag of wrought iron characteristics, substantially as described.

18. A spongy mass of wrought iron 120 formed of the granulated product of a steel-making process mixed with slag of wrought iron characteristics, said mass having the shape of the receptacle in which the mixture is formed, substantially as described. 125

19. A spongy mass of wrought iron 130 formed of the granulated product of a steel-making process mixed with slag of wrought iron characteristics, said mass having the shape of the receptacle in which the mixture

is formed and being of less density than that of hand puddled balls, substantially as described.

20. As a new article of manufacture, a shaped and compressed mass of wrought iron formed of the granulated product of a steel-making process mixed with slag of

wrought iron characteristics, said mass being of sufficient size to be rolled direct into slabs or billets without cutting and repiling, substantially as described.

In testimony whereof, I have hereunto set my hand.

JAMES ASTON.